

## UNITED STATES PATENT OFFICE

2,316,277

## DISCHARGE PRINTING ORGANIC DERIVATIVES OF CELLULOSE

Henry Charles Olpin and William Cyril Mc-Knight, Spondon, near Derby, England, assignors to Celanese Corporation of America, a corporation of Delaware

No Drawing. Application September 4, 1940,  
Serial No. 355,310. In Great Britain October  
20, 1939

12 Claims. (Cl. 8—64).

This invention relates to the production of pattern effects on textile materials of organic derivatives of cellulose, i. e. of cellulose esters or ethers. It is especially concerned with the production of such pattern effects on pale coloured grounds.

The range of dischargeable dyestuffs for pale shades, especially pale blue shades, on cellulose ester or ether materials is not entirely satisfactory owing to the difficulty of finding a really satisfactory colour meeting the various requirements of brightness of shade, fastness to light, dischargeability without hypersensitivity in pale shades to traces of discharging agent which may have accidentally come in contact with portions of the material other than those printed with the discharge composition, and resistance to steaming and general after processing, including the mild oxidation treatment which is commonly employed when using vat colours as illuminants. These requirements are not so difficult to meet in medium to full shades since any slight change in the ground shade, following the printing operation, would pass unnoticed, but the standard imposed for good discharge effects on textile materials coloured in pale shades is very searching.

It has now been found that satisfactory discharges with the usual sulphoxylate discharging agents may be obtained on cellulose ester or ether materials coloured in pale shades, particularly pale blue shades, with anthraquinone derivatives having direct affinity thereto, for example aminoanthraquinones, including N-substituted aminoanthraquinones. Since these anthraquinone derivatives meet the various requirements outlined above the pattern effects obtained are of great value.

According to the present invention, therefore, cellulose acetate or other cellulose ester or ether materials exhibiting pattern effects on pale coloured grounds are obtained by locally applying a sulphoxylate discharging agent to cellulose acetate or other cellulose ester or ether materials coloured in pale shades with an anthraquinone dyestuff having direct affinity thereto. As discharging agent there can be used, for example, zinc formaldehyde sulphoxylate or sodium formaldehyde sulphoxylate.

The possibility of obtaining in this way pattern effects on materials dyed with anthraquinone dyestuffs of the above type is most surprising, since 50 these dyestuffs have always been regarded as non-dischargeable. However, in pale shades, for example, the shades obtainable using up to 0.05% or even 0.1% of dyestuff, based on the weight of the goods, these anthraquinone derivatives have

been found to be sufficiently dischargeable with, for example, the normal alkaline discharge pastes to enable the discharged portions to be illuminated with vat or other colours without the residual colour of the reduced anthraquinone dyestuff appreciably affecting the brilliancy of the illuminant. Good white discharges can also be obtained by using a discharge paste containing a white pigment, for which purpose titanium dioxide is particularly suitable. On the other hand satisfactory discharges are not obtainable on fabrics dyed in full shades with anthraquinone derivatives, for example fabrics containing 0.25% of dyestuff based on the weight of the goods.

15 As illuminant in the production of coloured discharges there can be used any dyestuff resistant to the discharging agent and especially suitable for this purpose is a vat dyestuff.

For the ground shades the best results are obtained with 1:4-diaminoanthraquinones and 20 1-amino-4-hydroxy-anthraquinones in which one of the benzene nuclei is free from auxochromic substituents, especially amino and hydroxy groups, for example 1:4-dimethylaminoanthraquinone or 1-amino-4-cyclohexylaminoanthraquinone-2-carboxyamide. Anthraquinone derivatives of the type of 1:4-diethanolamino-5-hydroxyanthraquinone and 1:4-diethanolamino-5:8-dihydroxyanthraquinone are not usually so 25 satisfactory, since the colour of the reduced dyestuff left in the discharge portions may be more obtrusive. In contradistinction to anthraquinone vat colours which on reduction give the true leuco or meso dihydro compounds which may be reoxidised to the original shades, the anthraquinone dyestuffs having direct affinity for cellulose acetate give the more stable 2:3-dihydro-compounds, probably accompanied by scission of the amino group. They do not therefore reoxidise to the 30 original shade.

35 The invention is of particular importance in connection with the production of discharge effects on cellulose ester or ether materials, especially cellulose acetate materials, dyed in pale blue shades, since it is in these shades that the most difficulty is likely to be encountered when working with a truly dischargeable dyestuff. However, it may also be applied to materials dyed in pale shades other than pale blue, with anthraquinone dyestuffs or to materials dyed in a compound shade, part of which is due to an anthraquinone dyestuff and part to a truly dischargeable dyestuff, e. g. a dischargeable azo dye or a dischargeable nitro diarylamine dye or other dischargeable dyes having nitro groups as the sole

chromophores. For example, valuable discharges may be obtained according to the invention on materials dyed in pale green shades with a mixture of a blue anthraquinone dyestuff and a yellow dischargeable dyestuff of the above-mentioned type. As it is the blue constituent which usually gives trouble in this work when using a truly dischargeable blue dyestuff, it is found that discharges obtained upon materials dyed in pale green shades in this way are superior to those in which the dyestuff mixture consists of a truly dischargeable blue and a truly dischargeable yellow dyestuff.

The invention is illustrated by the following examples:

*Example 1*

Cellulose acetate fabric is dyed in a pale blue shade with either 0.025% of 1:4-di-(methylamino)-anthraquinone or 0.025% of 1-amino-4-cyanoxyhexylaminoanthraquinone - 2 - carboxyamide, based on the weight of the fabric, and then printed, using the following printing colours:

White: Parts

|                                             |     |
|---------------------------------------------|-----|
| Formosul (sodium formaldehyde sulphoxylate) | 5   |
| Titanium dioxide (1:1)                      | 20  |
| Egg albumen (1:1)                           | 20  |
| Gum tragacanth 6%                           | 45  |
| Water                                       | 10  |
|                                             | 100 |

Colours: Parts

|                               |      |
|-------------------------------|------|
| Dyestuff paste (see below).   |      |
| Formosul                      | 6.5  |
| Glycerine                     | 5    |
| Soda ash                      | 5.25 |
| Starch/British gum thickening | 45   |
|                               | 100  |

Water to make 100

The dyestuff used as illuminant may be any one of the following:

Yellow:

20 parts Indanthrene Yellow GOK  
(Schultz, Supplement 2, page 201).

Pale Blue:

2.2 parts Ciba Blue 2B (Colour Index No. 1184).

Green:

16 parts Paradone Yellow GC (an anthraquinone vat dyestuff).

4 parts Caledon Jade Green XS (Colour Index No. 1101 I. C. I. Shade Card "Caledon and Durindone Dyestuffs" 1937).

Red:

13.3 parts Durindone Scarlet YS (Schultz, Supplement 2, No. 1356).

6.7 parts Hydron Pink FF (Colour Index, page 355).

Pink:

1.1 parts Durindone Scarlet YS.  
0.55 part Hydron Pink FF.

After printing the pieces are dried, steamed and oxidised by hanging for 48 hours, washed off and soaped. The fastness of the ground shade is of a high order, both to light and to acid fading, and the pigment white also is of a satisfactorily high order of fastness to washing.

*Example 2*

Cellulose acetate material is dyed in pale green shades, using a mixture of either of the two anthraquinone dyestuffs mentioned in Example 1

and as dischargeable yellow dyestuff 2:4-dinitro-diphenylamine; 4:4' - diamino - 3:3' - dinitrodi-phenylmethane or the azo dyestuff from diazotised *p*-aminoacetanilide and *p*-cresol.

The materials are printed and after-treated as described in Example 1. The ground shade shows no appreciable modification.

Having described our invention, what we desire to secure by Letters Patent is:

1. Process for the production of patterned textile materials of an organic derivative of cellulose, which comprises locally discharging the ground color of such materials colored in pale ground shades with an amino anthraquinone dye having direct affinity therefor, by locally applying to the materials a composition containing a sulphoxylate discharging agent.

2. Process for the production of patterned textile materials of an organic derivative of cellulose, which comprises locally discharging the ground color of such materials colored in pale ground shades with a blue amino-anthraquinone dye having direct affinity therefor, by locally applying to the materials a composition containing a sulphoxylate discharging agent.

3. Process for the production of patterned textile materials of an organic derivative of cellulose, which comprises locally discharging the ground color of such materials colored in pale ground shades with a blue aminoanthraquinone dye having one of the benzene nuclei free from auxochromic substituents and having direct affinity for the materials, by locally applying to the materials a composition containing a sulphoxylate discharging agent.

4. Process for the production of patterned textile materials of an organic derivative of cellulose, which comprises locally discharging the ground color of such materials colored in pale ground shades with a blue aminoanthraquinone dye having one of the benzene nuclei free from auxochromic substituents and having direct affinity for the materials, by locally applying to the materials a composition containing a sulphoxylate discharging agent and a vat dye as illuminant.

5. Process for the production of patterned textile materials of an organic derivative of cellulose which comprises locally discharging the ground color of such materials colored in pale ground shades with a blue aminoanthraquinone dye having one of the benzene nuclei free from auxochromic substituents and having direct affinity for the materials, by locally applying to the materials a composition containing a sulphoxylate discharging agent and a white pigment.

6. Process for the production of patterned textile materials of an organic derivative of cellulose, which comprises locally discharging the ground color of such materials colored in pale ground shades with a mixture of a blue amino-anthraquinone dye having one of the benzene nuclei free from auxochromic substituents and a truly dischargeable dye, both dyes having direct affinity for the materials, by locally applying to the materials a composition containing a sulphoxylate discharging agent.

7. Process for the production of patterned cellulose acetate textile materials, which comprises locally discharging the ground color of such materials colored in pale ground shades with an amino anthraquinone dye having direct affinity therefor, by locally applying to the materials a composition containing a sulphoxylate discharging agent.

8. Process for the production of patterned cellulose acetate textile materials, which comprises locally discharging the ground color of such materials colored in pale ground shades with a blue amino-anthraquinone dye having direct affinity therefor, by locally applying to the materials a composition containing a sulphonylate discharging agent.

9. Process for the production of patterned cellulose acetate textile materials, which comprises locally discharging the ground color of such materials colored in pale ground shades with a blue amino-anthraquinone dye having one of the benzene nuclei free from auxochromic substituents and having direct affinity for the materials, by locally applying to the materials a composition containing a sulphonylate discharging agent.

10. Process for the production of patterned cellulose acetate textile materials, which comprises locally discharging the ground color of such materials colored in pale ground shades with a blue amino-anthraquinone dye having one of the benzene nuclei free from auxochromic substituents and having direct affinity for the materials, by locally applying to the materials a com-

position containing a sulphonylate discharging agent and a vat dye as illuminant.

11. Process for the production of patterned cellulose acetate textile materials, which comprises locally discharging the ground color of such materials colored in pale ground shades with a blue amino-anthraquinone dye having one of the benzene nuclei free from auxochromic substituents and having direct affinity for the materials, by locally applying to the materials a composition containing a sulphonylate discharging agent.

12. Process for the production of patterned cellulose acetate textile materials, which comprises locally discharging the ground color of such materials colored in pale ground shades with a mixture of a blue amino-anthraquinone dye having one of the benzene nuclei free from auxochromic substituents and a truly dischargeable dye, both dyes having direct affinity for the materials, by locally applying to the materials a composition containing a sulphonylate discharging agent.

HENRY CHARLES OLPIN.  
WILLIAM CYRIL MCKNIGHT.